

(No Model.)

J. BAYNES.

PROCESS OF ORNAMENTING VASES OR SIMILAR ARTICLES.

No. 468,591.

Patented Feb. 9, 1892.

Fig. 1.



Fig. 4.



Fig. 2.



Fig. 5.



Witnesses

Jno. G. Hinckley, Jr.

A. E. Finsmann.

Inventor

John Baynes,  
By his Attorneys  
John C. Freeman

# UNITED STATES PATENT OFFICE.

JOHN BAYNES, OF WESTCHESTER, ASSIGNOR OF ONE-FOURTH TO LOCKWOOD DE FOREST, OF OYSTER BAY, NEW YORK.

## PROCESS OF ORNAMENTING VASES OR SIMILAR ARTICLES.

SPECIFICATION forming part of Letters Patent No. 468,591, dated February 9, 1892.

Application filed January 8, 1887. Serial No. 223,783. (No model.)

*To all whom it may concern:*

Be it known that I, JOHN BAYNES, a subject of the Queen of Great Britain, residing at Westchester, in the county of Westchester and State of New York, have invented certain new and useful Improvements in the Manufacture of Articles Having Faces Ornamented by Metallic Patterns, of which the following is a specification.

10 My invention relates to the process of ornamenting vases or similar articles, substantially as hereinafter set forth.

In the drawings, Figure 1 is an elevation of a vase in part section and perspective view 15 of the pattern-plate, illustrating my improvement. Fig. 2 is a side view of a vase ornamented in accordance with my invention. Figs. 3 and 4 illustrate modifications of my process, and Fig. 5 illustrates an article composed 20 entirely of metal produced by my process.

For the purpose of describing my invention I shall refer to the manufacture of ornamental vases; but it will be understood that the invention may be employed in the manufacture 25 of various articles or parts of articles where a metal or alloy capable of being deposited electrically may be employed either for the purpose of forming the body of the article or part thereof or of forming an ornamental facing or partial facing thereto.

If it is desired to use the deposited metal as an overlayer upon a vase of pottery or similar material, I first properly prepare the surface of the vase A, so that it will receive a deposit of metal by electricity from a suitable 35 solution by coating it with a base or foundation film of composition, such as wax and plumbago, and I then place it in such solution and apply the deposit in a manner too

40 well known to need description, the said deposit constituting a continuous overlying film 2 of a thickness which may be varied to any desired extent. Upon the surface of film 2 is then applied a coating of any suitable resist 45 sensitive to light, the said coating being indicated by dotted lines 3, Fig. 1 of the drawings, and light is then thrown through a pattern-plate B onto the sensitive face of the coating, thereby rendering such portions as 50 are exposed to the actions of the light soluble or insoluble, according to the character of the

coating. The soluble portions of the coating are now dissolved, leaving the pattern traced by the insoluble portions, and the article is then immersed in an acid bath, which will 55 etch into or through the electro-deposit film wherever the same may be exposed, after which the article is removed and the resist is scraped or otherwise removed, leaving upon the surface of the article an ornamental pattern of the electro-deposited metal. The resist coating 3 need not in all cases be sensitive to light, as an ordinary acid-resist of asphaltum 4 may be employed in connection with a stencil 5, applied thereto, the exposed portions of the resist being removed by abrasion 60 by means of a brush or by the action of a solvent, as turpentine or naphtha, carried by a brush or sponge. A second coating of a different metal may be applied upon or in any 65 desired position in relation to the pattern formed by the first coating to secure a more elaborate ornamentation of the article. This second pattern is deposited by first coating the article having the first pattern thereon 70 with a film of wax and plumbago, electro-depositing a second base or foundation film of another metal over the entire surface, and then etching through the second film of metal 75 in the same manner as before. If, for instance, the vase A, Fig. 2, be a porous vase, upon which the flower pattern has been deposited of one metal—say silver—the second pattern or ornamentation, representing flying birds or insects, is deposited in like manner 80 in gold or nickel.

While I may use any of the resists and solvents known to those skilled in the art, I have found a resist—such as is described in my Patent No. 282,485, dated August 7, 1883— 90 consisting of, say, ninety parts of asphaltum, eighty parts of oil of turpentine, and ten parts gum-copal, and the parts unaffected by light may be removed by applying a solvent, as turpentine, in any usual manner. The time of 95 exposure to light, of course, will depend upon the composition used, the condition of the light, and the character of the work to be done, and may vary from two hours, more or less.

The body of the article may be made entirely of the electro-deposited metal by first 100 forming a pattern of soluble or friable mate-

rial—as, for instance, plaster-of-paris 6—coating it with plumbago, depositing a heavy film of metal 7—say copper—thereon, then coating the latter with a resist 8, forming the pattern 5 on the resist, and etching through the same and completely through the body metal (see Fig. 5) in the same manner as hereinbefore described, the model being then broken or removed by a suitable solvent, leaving a hollow 10 perforated shell. The first base or foundation coating or film of wax and plumbago is also removed by dissolving it in a suitable solution or otherwise, leaving the electro-deposited coating surrounding the body of the 15 vase or other vessel, but independent of it.

It will be evident that my improved method of ornamenting articles may be applied in connection with various metals capable of electro-deposit in the manufacture of various 20 different articles or parts of articles, like tiles and similar articles.

Without limiting myself to the precise manipulations herein set forth or to the use of the special materials specified, I claim—

25 1. The process of ornamenting vases or similar articles having ornamental metal patterns upon their faces, which consists in first coating the articles with a film of wax and plumbago, then coating the entire face of the 30 body portion of the article with a film of the ornamenting metal by electro-deposition, then applying a coating of resist susceptible to the action of the light, then acting upon the re-

sist by rays of light through a pattern-plate, 35 then removing the soluble portions of the resist and etching through the ornamenting metal at the exposed parts, then removing the resist from the protected parts of the metal, and finally removing the wax and plumbago, substantially as set forth.

2. The process of ornamenting vases or similar articles having ornamental metal patterns upon their faces, which consists in first applying a base or foundation coating of wax and plumbago to the body of the article, then 45 coating the entire face of the body portion of the article with a film of the ornamenting metal by electro-deposition, then applying a coating of resist, subjecting it to the rays of light through a pattern-plate and removing 50 the soluble portions thereof, then etching through the ornamenting metal at the exposed parts, then applying a second foundation-coating of wax or plumbago, then applying a second metallic coating of a different metal 55 upon said face, and repeating the operations to complete the ornamentation, and finally removing the base-coatings, substantially as set forth.

In testimony whereof I have signed my 6c name to this specification in the presence of two subscribing witnesses.

JOHN BAYNES.

Witnesses:

BERNARD J. KELLY,  
LOCKWOOD DE FOREST.